

March 11, 1952

C. J. DIPPEL ET AL

2,588,811

PROCESS OF DRYING GELATINE LAYERS

Filed May 2, 1947



FIG. 1.

FIG. 2.

INVENTORS.  
CORNELIS JOHANNES DIPPEL  
JAN ANTHONY LELY  
BY JOHANNES ALOIUSIUS MARIA DICKHOFF  
*Jan A. Dippel*  
AGENT.

## UNITED STATES PATENT OFFICE

2,588,811

## PROCESS OF DRYING GELATINE LAYERS

Cornelis Johannes Dippel, Jan Anthony Lely, and  
 Johannes Aloysius Maria Dikhoff, Eindhoven,  
 Netherlands, assignors to Hartford National  
 Bank and Trust Company, Hartford, Conn., as  
 trustee

Application May 2, 1947, Serial No. 745,396  
 In the Netherlands June 1, 1946

4 Claims. (Cl. 34—1)

1

In drying gelatine layers, for example in manufacturing photographic material, great difficulty is encountered in that gelatine can only be dried very slowly. The installations for making photographic material in which a photo-sensitive gelatine emulsion is provided on a substratum thus become of very large size and hence very expensive. The avoidance of the formation of dust in such large spaces of several tens of meters in length, which is absolutely necessary for making good photographic material, increases the cost to a considerable extent. Furthermore, the usual heating by means of heated dry air has a poor efficiency. Similar difficulties arise in manufacturing gelatine layers which do not comprise photosensitive compounds such, for example, as gelatine layers which are intended for recording sound by mechanical means, for example by cutting a sound track film or record.

The present invention relates to a process of drying gelatine layers which permits drying to be effected at a considerably greater speed with the use of equipment of very small size.

According to the invention, gelatine layers are dried by heating in an electric field of high frequency.

Whereas in drying a coagulated gelatine emulsion by means of heated dry air, as has been usual hitherto, drying may take place only very slowly since otherwise the gelatine melts and inhomogeneous layers are obtained. It has been found that the use of high-frequency drying permits the temperature of the gelatine layer to exceed its melting point without any harmful consequences for the homogeneity of the gelatine layer being involved.

This affords the possibility of greater speed in the drying process. According to the invention an aqueous gelatine layer which, after drying, has a thickness of 100 microns at the most is subjected to an electric field while passing a stream of gas over the gelatine for dissipating the water vapour produced, said field being of such frequency and strength that the water is removed within five minutes. A treatment of five minutes at the most means that any point of the layer is subject to the field for five minutes at the most.

For a better understanding of the invention it is pointed out that the reason why melting of the gelatine layer need not necessarily result in any unevenness is probably due to the fact that the water which is at first evaporated is rapidly removed so that partly dried gelatine of low water content follows almost immediately. This gelatine upon melting yields a mass of such

2

viscosity that flows or the like which might lead to troublesome unevennesses no longer occur in it. Since the gelatine treated according to the invention is dried, at least initially, in the molten state it is not necessary for the gelatine emulsion, after being poured out on a substratum to form a layer, to coagulate before drying, contrary to the drying methods which have been usual hitherto. It is further pointed out that a gelatine emulsion of the kind utilized for pouring out a layer of uniform thickness usually contains from 80% to 90% by weight of water. If such an emulsion is caused to coagulate by cooling and subsequently heated up, it melts below a temperature of 30° C. to form a thin fluid mass. The water content decreases as the melting point increases. An emulsion which has been dried to a water content of about 50% produces a molten mass which exhibits at 50° C. a viscosity such that no troublesome flaws occur in it. Gelatine layers of photographic films are dried to a water content of about 15%. With such a water content the layers are about ten times thinner than in the freshly-coagulated undried state.

It is evident that the speed of drying is dependent on the thickness of the gelatine layer. Layers of a thickness of about 50 microns, such as are used for cutting mechanical sound records, for example sound film records exhibiting so-called variations in width, require a drying time longer than that for layers of from 15 to 20 microns such as are used for the ordinary photographic silver halide gelatine material. According to the invention, the last-mentioned layers are adapted to be dried within half a minute.

Heating of the gelatine layer is preferably effected by means of an electric field generated between filamentary or rod-shaped electrodes which are arranged parallel to the surface of the layer and along which the gelatin layer is guided in such manner that the lines of force of the field extend through the material substantially in the direction of movement. With such an arrangement of the electrodes the lines of force extend over a comparatively long distance through the layer itself and over only a small distance through the medium, for example air, between the electrodes and the material to be dried. This results in an increase of the efficiency of the field so that a great amount of heat may be generated in the gelatine layer by means of small equipment and a high-frequency generator of low power.

Although with the said arrangement of the

electrodes the strength of the field in the direction of movement of the material is not constant, the result of the treatment in this direction is homogeneous provided that the movement takes place at constant speed. The homogeneity in the transverse direction, normal to the direction of movement, may be controlled by the use of electrodes the length of which is greater than the width of the material.

The arrangement of the electrodes is preferably such that, on passing the electrodes, the gelatine layer is subjected to a field of gradually decreasing strength, since as the drying process is proceeding and the gelatine contains less water, the water is driven out of the gelatine more slowly, probably due to the fact that a thin layer of poor transmitting capacity forms on the surface of the gelatine layer. Consequently, the risk of undue heating of the gelatine increases. Although the gelatine in this drying stage exhibits a viscosity such that flows in the gelatine need practically not be feared, there is in this case a risk of the formation of vapour and hence of bubbles in the gelatine layer. A gradually decreasing field may be obtained by a gradual increase of the distances between the electrodes between which the field is generated, by a decrease of voltage, and so on.

As an alternative, weaker heating in the last stage of the drying process may be obtained by treating the gelatine layer in this stage with cold air.

Local overheating as a result of locally greater intensity of the field is avoided by control of the rate at which the gelatine layer is guided through the field so that the layer is subject to these points of higher field intensity for a short time only. The rate which is preferably used is about 0.5 metre per minute.

The gelatine layer may be guided between the electrodes in the horizontal position, or in the inclined, for example vertical, position. Any guide rollers or guide paths which may be provided in the electric field are required to consist of material of low dielectric losses so that they are not unduly heated. There need be no fear of combustion of the substratum, e. g. nitrocellulose for the gelatine due to electrostatic charges generated by friction on the rollers, since with the use of the invention the atmosphere in the drying space is not required to be as dry as in the usual processes, in which heating and drying take place by means of heated dry air.

The amount of gas, for example air, which is guided along the gelatine layer for the dissipation of the water vapour is preferably such as to be just sufficient for the absorption of the expelled water vapour without becoming oversaturated. This affords the advantage that the amount of air that is directed over the gelatine may be as small as possible so that the risk of contamination of the gelatine layer by dust particles is reduced. The amount of air is preferably 100% more than that which is required for the dissipation of the water vapour.

In the usual process of drying gelatine the amount of air flowing along is considerable in order to enhance as much as possible the vaporisation of water brought about by the slightly heated and very dry air. With such large amounts of air flowing along the gelatine the risk of contamination by dust particles is very great.

According to the invention, the air is preferably guided along the material in the same direc-

tion as that in which the material is moved. The air thus first comes into contact with the moistest gelatine from which a great amount of water is required to be absorbed quickly and at which the temperature is required to be lowest. During flowing through the heating device the temperature of the air increases. This is not objectionable since the melting point of the gelatine with which it is in contact also rises as the water is driven out and the viscosity of the melted and partly dried gelatine is such that unevenness due to flaws in the gelatine do not arise. On the contrary, this heating of the air is advantageous since the capacity of air to absorb water vapour increases as the temperature rises. The air thus remains capable of absorbing water vapour from the gelatine, which is advantageous since the water vapour may thus be absorbed by a small amount of air.

It is further pointed out that in drying gelatine layers in an electric field the heat is largely generated in the gelatine and the substratum is hardly heated due to the fact that the dielectric losses of a dry substratum are considerably lower than those of a wet gelatine layer.

The invention is advantageously applicable not only to drying gelatine layers that are freshly applied but also to drying gelatine layers which, after drying, are moistened again, for example photographic material which is developed, fixed and rinsed.

The invention will be described in connection with the following example and the accompanying drawing in which:

Fig. 1 shows one form of apparatus for drying film; and

Fig. 2 shows another form of apparatus for drying film.

#### Example

A band of nitrocellulose having a width of 16 mms. and a thickness of 135 microns has applied to it a gelatine layer by treatment with a solution containing 20% of gelatine at about 35° C. and by coagulation of the emulsion. Subsequently, the layer is guided in the vertical direction from below to above, at a speed of 0.7 meter per minute, through an electric field having a frequency of 15 megacycles/sec. and a power of 80 watts, the layer being dry within 15 seconds. About 35 liters of air per minute at the ambient temperature is directed along the layer. The thickness of the layer in the dried state is about 25 microns. The electrode system used for generating the electric field is shown diagrammatically in the accompanying drawing. Reference numeral 1 indicates the nitrocellulose band which is provided with a gelatine layer and which is moved from below to above. The electrodes 2 which are arranged to be mutually shifted are rod-shaped and have a diameter of 3.5 mms. and a length of 20 mms. All the electrodes on the same side of the band are interconnected in a conductive manner and are energized by an r-f oscillator 3. The lowermost seven electrodes are at a distance of 2 mms. from the band and exhibit a mutual spacing of 10 mms. The remaining electrodes are at a distance of 4 mms. from the band and exhibit mutual distances of 30 mms. The electrode system is arranged in a tube 4 consisting of material of low dielectric losses through which a stream of air is passed by means of an exhaust fan 5 in Fig. 1 or by means of a blower system comprising an intake fan 6 and an exhaust fan 5 in Fig. 2.

What we claim is:

1. A process of drying gelatine layers, having a thickness when dried of less than approximately 100 microns comprising the steps of subjecting the gelatine layer containing water to an alternating electric field of high frequency having an intensity at which the gelatine is heated to a temperature at which it melts and the water removed therefrom within five minutes, and passing a gas stream over the gelatine layer to remove the water vapor expelled from the wet gelatine layer.

2. A process of drying gelatine layers, having a thickness when dried of less than approximately 20 microns comprising the steps of subjecting the gelatine layer containing water to an alternating electric field of high frequency having an intensity at which the gelatine is heated to a temperature at which it melts and the water removed therefrom within one-half a minute, and passing a gas stream over the gelatine layer to remove the water vapor expelled from the wet gelatine layer.

3. A process of drying gelatine layers, having a thickness when dried of less than approximately 100 microns comprising the steps of passing the gelatine layer containing water through an alternating electric field of high frequency having an intensity at which the gelatine is heated to a temperature at which it melts and the water removed therefrom within five minutes at a speed exceeding one-half meter per minute, and passing a gas stream over the gelatine layer to remove the water vapor expelled from the wet gelatine layer.

4. A process of drying gelatine layers, having a thickness when dried of less than approximately

100 microns comprising the steps of passing the gelatine layer containing water through an alternating electric field of high frequency having lines of force extending substantially parallel to the direction of motion of the layer and having an intensity at which the gelatine is heated to a temperature at which it melts and the water removed therefrom within five minutes at a speed of at least one-half meter per minute, and passing a gas stream over the gelatine layer to remove the water vapor expelled from the wet gelatine layer.

CORNELIS JOHANNES DIPPEL.

JAN ANTHONY LELY.

JOHANNES ALOYSIUS MARIA DIKHOFF.

#### REFERENCES CITED

The following references are of record in the file of this patent:

#### UNITED STATES PATENTS

| Number    | Name         | Date          |
|-----------|--------------|---------------|
| 2,042,145 | Darrah       | May 26, 1936  |
| 2,226,871 | Nicholas     | Dec. 31, 1940 |
| 2,231,457 | Stephen      | Feb. 11, 1941 |
| 2,291,807 | Hart, Jr.    | Aug. 4, 1942  |
| 2,402,609 | Brabander    | June 25, 1946 |
| 2,459,623 | Cohoe et al. | Jan. 18, 1949 |
| 2,473,251 | Hsu          | June 14, 1949 |

#### FOREIGN PATENTS

| Number  | Country | Date         |
|---------|---------|--------------|
| 691,038 | Germany | May 15, 1940 |